

Patented Oct. 23, 1923.

1,471,846

# UNITED STATES PATENT OFFICE.

HENRY H. HINDSHAW, OF ST. PAUL, MINNESOTA, ASSIGNEE TO HINDSHAW ENGINEERING & DEVELOPMENT CO., OF ST. PAUL, MINNESOTA, A CORPORATION OF MINNESOTA.

## HEAT-INSULATING MATERIAL.

No Drawing.

Application filed December 7, 1921. Serial No. 520,588.

To all whom it may concern:

Be it known that I, HENRY H. HINDSHAW, a citizen of the United States, residing at St. Paul, in the county of Ramsey and State of Minnesota, have invented certain new and useful Improvements in Heat-Insulating Materials; and I do hereby declare the following to be a full, clear, and exact description of the invention, such as will enable others skilled in the art to which it appertains to make and use the same.

This invention relates to a heat insulating material and the process of making the same. Such heat insulating materials are now widely used for lining walls of cold storage and other chambers, covering pipes and as a covering for various surfaces to retard heat radiation.

It is an object of this invention to produce a heat insulating material of high efficiency by the use of vegetative mosses, particularly the mosses belonging to the genus Sphagnum, which mosses will be coated and cemented or bound together by peat.

It is a further object of the invention to mix the materials together in the proper proportion and to knead and manipulate the mixture so that the moss will be thoroughly coated with the binding material or peat.

These and other objects of the invention will be more fully set forth in the following detailed description.

The mosses of the genus Sphagnum grow in large abundance and over wide areas in this country and grow in wet or swampy ground where, by the annual decay and deposit, they form the principal material of peat bogs. This moss occurs as such, of course, at the top of the peat bog and varies in thickness at different places averaging, possibly a depth of twenty four inches. While the material of the present invention is preferably made from Sphagnum moss, yet mosses of genus Hypnum may also be effectively used. The leaves of the Sphagnum moss are composed of layers of minute open ended cells and when the leaves are coated with a film of material which solidifies and the material is dried, the result is a plurality of closed gas filled chambers. It is well known that the heat insulating properties of most materials are due to the same containing a plurality of gas or air filled cavities. The mosses herein used therefore are particularly adapted for use in making a

heat insulating material.

To properly coat the leaves and stems of the moss and to form a binder for holding the material together, a well humified peat is used. This peat can be obtained from the same locality and deposit as the moss. While the moss occurs at the surface, it is necessary to go down to a depth of ten or twelve feet to secure a suitable peat, as it is necessary that the peat be well ripened or humified. Such peat, when first taken from the bog contains a great deal of moisture and has pronounced adhesive properties due to the fact that the protein therein is then in the form of pectose. When this peat has once been dried it undergoes an organic change so that it can not afterwards again be brought to its adhesive condition, said change consists in the pectose being changed into pectin. The peat when thus taken from the bog and when in its natural condition forms an admirable substance for coating and binding the moss together.

In producing the insulating material, the moss is first harvested or gathered from its natural bed and any hard wood or other foreign substances mixed therewith are separated, the moss being loosened or picked over carefully by hand or any suitable apparatus for this purpose. After the moss has thus been separated from foreign substances, if it is not already sufficiently moistened, water will be added so that the moss is in a thoroughly moistened condition. The moss is then mixed with a quantity of raw peat. As stated, at this time, the peat also contains a great deal of moisture. The proportions of the two quantities vary considerably, depending upon the use to which the resulting material is to be put. Generally, the weight of the peat will be from five to twenty-five percent of the weight of the moss used, these weights referring to the dry or anhydrous condition of the materials. After the moss and peat have been mixed, they are thoroughly kneaded or mixed together and during this process the moss will be somewhat disintegrated. The leaves and stems of the moss, during this kneading operation, will become thoroughly coated with a thin layer of peat which will form a film sealing the open ends of the cells thereof. This kneading operation can be performed by various apparatus but can be efficiently carried out in the well known chas-

ing mill having a revolving pan in which rest rolls having on their peripheries transverse ridges or corrugations. This kneading process is continued until the coating of 5 the leaves above referred to has been thoroughly accomplished. The product resulting from this part of the process is a pulp of plastic consistency. This pulp is then 10 molded into sheets of the desired thickness, either by rolling or by the use of mold boxes.

The material is then dried by treatment 15 in a partial vacuum or any other suitable way until it is in a hard solid condition. 15 This material can then be cut into sheets, blocks or boards, as desired. Such material is light, capable of being readily cut and possesses considerable tensile strength, so 20 that the same can be nailed into position as an ordinary board. Owing to the large de- 25 posits of this moss and peat and their near- 30 ness to the surface, this insulating material can be very cheaply made. As above stated, the amount of peat used will vary some- 35 what, according to the use of the material. If a very light substance is desired, for 40 lining refrigerators, etc., just enough peat will be used to act effectively with the moss. Where a greater strength and weight are 45 desired, however, as where the material will be used in flooring or building structures, a 50 greater percent of peat can be added.

This material is also well adapted for 35 fire proofing and water proofing treatment. It has been found that by adding to the mixture of moss and peat certain proportions of 40 mineral substances, a hard porous product is obtained having the desirable heat insulating qualities and yet forming an efficient sub- 45 stance for the flooring or wall construction in refrigerator cars, and similar uses, and is susceptible of an ornamental finish making it 50 desirable for ornamental wainscoting in building structures and similar uses. The surface of the material can, of course, be coated with well known water proofing materials. Furthermore, the material can be reinforced by fibrous or metallic materials either with the object of ultimate strength, 55 or as a guide to its form or setting or solidifying.

The material herein disclosed has been

found, in practice, to be very efficient for the purposes desired.

It will, of course, be understood that 55 various changes may be made in the various steps of manufacture, the proportions of the materials and details of the operations, without departing from the scope of applicant's 60 invention, which, generally stated, consists 65 in the matter herein disclosed and set forth in the claims.

What is claimed is:

1. An insulating material composed of 65 particles of moss bound together by peat.
2. An insulating material composed of 70 particles of moss of cellular structure coated with and bound together by peat.
3. An insulating material comprising 75 Sphagnum moss, the leaves of which are coated and bound together by a binder of humified peat.
4. A dry hard insulating material com- 80 posed of disintegrated Sphagnum moss coated and bound together by a humified peat binder.
5. The process of producing an insulating material which consists in mixing moist moss with raw peat, kneading the sub- 85 stances to thoroughly mix the same and to coat the leaves and stems of the moss with peat to form a plastic pulp, and then drying the mixture to form a hard solid substance.
6. The process of producing an insulating 90 material which consists in providing Sphag- 95num moss, loosening and moistening the same, mixing therewith substantially one-ninth of the amount, by weight of the dry materials, of raw humified peat, mixing and kneading the materials to thoroughly coat the parts of the moss with the peat, and to form a plastic pulp, molding said pulp into sheets and drying the product to produce a dry solid material.
7. The process of producing a dry hard 95 insulating material consisting in disintegrating vegetable fiber, mixing and coating the same with undried peat which is in its natural condition, whereby the particles of 100 fiber are bonded by the peat, and then drying said mixture whereby a tough hard product is obtained.

In testimony whereof I affix my signature.

HENRY H. HINDSHAW.